

# United States Patent [19]

Gibson

[11] Patent Number: 4,816,297

[45] Date of Patent: Mar. 28, 1989

- [54] **METHOD OF POWDER COATING THE INSIDE OF PIPES WITH A CONTINUOUS FILM OF PLASTIC MATERIAL**

[76] Inventor: **Jack E. Gibson, 4905 Pepperidge Pl., Odessa, Tex. 79761**

[21] Appl. No.: **786,818**

[22] Filed: **Oct. 11, 1985**

#### Related U.S. Application Data

- [60] Continuation of Ser. No. 516,661, Jul. 21, 1983, abandoned, which is a continuation of Ser. No. 180,191, Aug. 22, 1980, abandoned, which is a division of Ser. No. 862,261, Dec. 20, 1977, Pat. No. 4,243,699.

[51] Int. Cl.<sup>4</sup> ..... B05D 1/12; B05D 7/22

[52] U.S. Cl. ..... 427/183; 427/233;  
427/234; 118/312; 118/DIG. 10; 118/308

[58] Field of Search ..... 118/620, 312, 308, 320,  
118/322, 326, DIG. 10; 427/181, 182, 183, 195,  
232, 233, 234, 238

## [56] References Cited

## U.S. PATENT DOCUMENTS

- |           |        |                   |           |
|-----------|--------|-------------------|-----------|
| 3,207,618 | 9/1965 | DeHart .....      | 427/183 X |
| 3,974,306 | 8/1976 | Inamura .....     | 427/183   |
| 3,982,050 | 9/1976 | Kato et al. ..... | 427/183   |
| 4,089,998 | 5/1978 | Gibson .....      | 427/183   |

## FOREIGN PATENT DOCUMENTS

295268 3/1966 Australia ..... 427/182

*Primary Examiner*—Shrive Beck  
*Attorney, Agent, or Firm*—Marcus L. Bates

[57] ABSTRACT

A method of powder coating the inside of tubular goods, such as oilfield pipe and the like, by connecting one end of the pipe to a means for producing a flow of compressible gases therethrough. The other end of the pipe is open to atmospheric pressure. A valve means is connected for controlling the flow of air through the container which holds a single charge of plastic powder. The charge of powdered plastic is isolated upstream of the pipe inlet. The charge is of sufficient size to coat the entire inside peripheral wall surface of the pipe with a substantial uniform coating of plastic. The pipe is heated above the softening temperature of the plastic and axially rotated, so that when the valve is opened, air flows through the container, into the pipe, and establishes a pressure gradient across the entire length of the pipe. This action causes the captured charge of plastic to form a pocket of dispersed plastic particles which is forced to flow through the pipe by the air flow. The plastic particles are deposited and fused to the hot rotating inner surface of the pipe.

**5 Claims, 2 Drawing Sheets**



FIG. I



FIG. 2



FIG. 4



FIG. 3



FIG. 5



FIG. 6



FIG. 7



**METHOD OF POWDER COATING THE INSIDE  
OF PIPES WITH A CONTINUOUS FILM OF  
PLASTIC MATERIAL**

**REFERENCE TO RELATED APPLICATIONS**

This patent application is a continuation of Ser. No. 516,661 filed July 21, 1983, now abandoned; which in turn is a continuation of Ser. No. 180,191 filed Aug. 22, 1980, now abandoned; which was a division of Ser. No. 862,261 filed Dec. 20, 1977, now U.S. Pat. No. 4,243,699. U.S. Pat. No. 4,243,699 was copending with Ser. No. 704,964 filed July 13, 1976, now U.S. Pat. No. 4,089,998, issued May 16, 1978, and Ser. No. 795,127 filed May 9, 1977, now U.S. Pat. No. 4,122,798 issued Oct. 31, 1978. A reissue patent application Ser. No. 06/335,162 was filed Dec. 28, 1981 based on U.S. Pat. No. 4,243,699.

**BACKGROUND OF THE INVENTION**

The difficulty of applying uniform plastic coatings to the interior of pipe and other tubular goods increases in proportion to the diameter and length of the pipe. Epoxy is one of the most satisfactory plastic coatings for oilfield pipe. An epoxy coating preferably is applied in powdered form to the heated, rotating pipe interior, where the plastic is fused into a continuous film and thereafter the pipe is cooled as the film solidifies to provide a superior coating which protects the metal pipe surface from chemically reacting with the material flowing therethrough, thereby elongating the life of the pipe.

In my co-pending patent application Ser. No. 704,965, filed July 13, 1976, now U.S. Pat. No. 4,089,998 issued May 16, 1978, there is taught a novel process by which pipe is coated in the above manner. The present patent application provides improvements over this previous process. As pointed out therein, the inside peripheral wall surface of a heated pipe can be coated in a superior manner by passing a pocket comprised of a dense, fluidized bed of plastic through the interior of a heated, rotating pipe so that the hot interior surface of the pipe is contacted by the plastic particles, whereupon the particles fuse to the inside wall of the pipe, thereby causing a uniform, continuous plastic coating to be achieved which was superior to other coatings known at that time. Following this discovery, Applicant has found other useful and novel processes by which the pocket of dispersed plastic particles can be transferred into and forced through the pipe in order to achieve an unexpected coating advantage. This new discovery is especially beneficial in coating large diameter pipe of considerable length, and this new process is the subject of this patent application.

**SUMMARY OF THE INVENTION**

A method of powder coating the inside surface of a pipe with a uniform continuous coating of plastic. The pipe is heated above the softening temperature of the plastic particles and rotated about its longitudinal axis. In one embodiment of the invention, a valve means connects one end of the pipe to be coated to a source of compressed gas while the other end of the pipe is left open to atmospheric pressure. A pocket of plastic is isolated upstream of the pipe inlet and downstream of the valve. The quantity of plastic contained within the pocket is about ten per cent greater than the weight of the coating to be formed. The heated pipe is rotated

about the longitudinal axial centerline thereof and the valve means is opened, whereupon, as the pocket of plastic is forced to move through the entire length of the pipe, the particles thereof progressively contact and deposit upon the inner pipe surface where they are fused into a continuous plastic film.

As the entire pocket of powdered plastic is blown from the upstream isolated location, through the heated spinning pipe, and, as the pocket of plastic particles flows from the inlet to the outlet end of the pipe, most of the particles contained within the pocket contact the pipe wall and fuse into a uniform continuous film of plastic, with a small excess of the powdered plastic exiting from the pipe outlet.

More specifically, a quantity of powdered plastic is placed within a chamber between two series connected valve means, with the upstream valve leading to the compressed gas source and the downstream valve leading to the inlet end of the pipe. The two valves are simultaneously opened, thereby entraining or fluidizing the isolated quantity of plastic powder which is forced to flow as a fluidized pocket of finite length into and through the heated pipe, where the particles contact and fuse to the rotating heated inner pipe surface.

In another embodiment of this invention, the mass flow through the heated rotating pipe is augmented by the placement of an air inlet upstream of the inlet end of the pipe and downstream of the isolated but dormant charge of plastic. This augmented air supply initially establishes a mass flow through the pipe so that when the blow air behind the pocket is established, there is no inertia of the system which must be overcome, and accordingly, improved flow characteristics of the system are realized.

In still another embodiment of the present invention, the inlet end of the apparatus containing the dormant charge of plastic is left opened to atmosphere while suction is applied to the outlet end of the pipe. The suction provides the only means by which the pocket of fluidized plastic particles is formed and transferred through the hot rotating pipe.

A primary object of this invention is the provision of a method of coating the interior of a pipe with a continuous uniform film of plastic by placing a quantity of the powdered plastic upstream of the heated pipe and flowing the powder through the pipe so that most of the powdered plastic contained within the pocket contacts the heated pipe wall and fuses into a uniform coating.

Another object of this invention is to plastic coat the interior of tubular objects by isolating a quantity of plastic particles upstream of a heated pipe and forcing the charge through the pipe by applying air pressure upstream of the charge while the outlet end of the pipe is open to atmospheric pressure.

Still another object of this invention is the provision of a process for internally coating pipe with a continuous film of plastic by forming a dormant charge of plastic particles upstream of a heated pipe and thereafter forcing the charge to flow through the pipe so that most of the particles contained within the charge contact the hot pipe wall while the charge is in the act of flowing through the pipe, thereby fusing the particles into a continuous film which is substantially uniform along the entire length of the pipe.

Another and still further object of this invention is a method of powder coating the inside of a pipe by forming a fluidized pocket of plastic particles upstream of a

heated pipe and flowing the pocket through the pipe under positive pressure and rotating the pipe as the particles contact and fuse to the pipe wall, so that a continuous plastic film extends for substantially the entire length of the pipe.

Still another and further object of this invention is the provision of a method of coating the inside peripheral wall surface of a pipe by forming an isolated charge of plastic upstream of the pipe inlet, applying a suction at the outlet end of the pipe, thereby forcing the pocket of plastic to be entrained into a pocket which is a dense fluidized bed of finite length. As the formed pocket of plastic particles flows through the pipe, the individual particles thereof progressively contact the pipe wall and fuse into a continuous uniform layer which coats substantially the entire length of the pipe. Most of the plastic which forms the pocket is fused into a coating as the pocket is forced through the entire length of the pipe.

These and various other objects and advantages of the invention will become readily apparent to those skilled in the art upon reading the following detailed description and claims and by referring to the accompanying drawings.

The above objects are attained in accordance with the present invention by the provision of a method for use with apparatus fabricated in a manner substantially as described in the above abstract and summary.

#### BRIEF DESCRIPTION OF THE DRAWINGS

FIG. 1 is a schematical representation of process and equipment according to the present invention;

FIG. 2 is an enlarged, fragmented, part cross-sectional view of part of the apparatus seen disclosed in FIG. 1;

FIG. 3 is an enlarged, cross-sectional view taken along line 3-3 of FIG. 2;

FIG. 4 is similar to FIG. 2 and discloses another embodiment thereof;

FIG. 5 is a schematical representation of another embodiment which discloses the process according to the present invention;

FIG. 6 is a fragmentary, enlarged, cross-sectional representation of a pipe which is in the act of being coated according to this invention; and,

FIG. 7 is a fragmented, part cross-sectional representation of apparatus for use in conjunction with still another embodiment of this invention.

#### DETAILED DESCRIPTION OF THE PREFERRED EMBODIMENTS

In the embodiment of the invention disclosed in FIG. 1, a pipe rack 10 successively supplies pipe 18 to a cleaning apparatus 12, such as, for example, sand blasting or shot peening using prior art equipment. The clean pipe is next heated in an oven 14 by means of a burner device 15, whereupon the heated pipe proceeds to station 16 where it is plastic coated according to this invention.

The station 16 includes a pipe spinning apparatus 19 which spins the pipe about its longitudinal axial center-line at a rotational speed of about 100 to 150 rpm as a charge of powdered plastic is forced therethrough. The exact rotational velocity varies with the diameter of the pipe which must spin at a speed which enables the deposited plastic particles to contact the pipe wall and thereafter spread out into a smooth, uniform film as it hardens or solidifies due to atmospheric cooling of the coating.

The coated pipe is next transferred into an oven 20 which is heated by a burner means 21. The soaking or subsequent heating station 20 is sometimes omitted, depending upon the chemical characteristics of the plastic powder. The coated pipe is inspected at station 22 and racked at 23.

Adapter devise 25 of FIGS. 1, 2, and 4 has a pipe receiving end 24 which is removably attachable to the inlet end of the spinning pipe as suggested by line 24', the details of which are more specifically disclosed in my co-pending patent application Ser. No. 704,965 filed July 13, 1976, now U.S. Pat. No. 4,089,998 issued May 16, 1978. Flexible hose 26 connects the adapter 60, and forms part of the pocket-forming apparatus 28. The pocket-forming apparatus includes a longitudinally disposed housing 29 having an axial passageway formed therethrough which is divided into a plurality of chambers. Pipe 30 leads to a source of compressible fluid, preferably air, and includes N.C. (ie, normally closed) valve device 31 which rapidly opens and closes in response to energization of solenoid 32. The inlet pipe diverges at 33 into an enlarged, charge-containing enclosure 36 of sufficient size to contain a single charge. Hopper 34 contains an ample supply of powdered plastic material of a composition which is suitable for use in conjunction with this invention, such as exemplified by the following products, and referred to in the claims as a synthetic, resin material:

- 30 (1) Corvel Polymer ECA-1446 TAN 2818 epoxy;
- (2) Corvel Polymer ECA-1456 TAN 2862 epoxy-phenolic;
- (3) M & T 8500 C012 TAN epoxy.

In the various figures of the drawings, the valve device 37 is spaced from valve device 31 and is moved from the N.C. to the open position by the action of a solenoid 38. N.O. and N.C. solenoid actuated valves 39 and 41, respectively, are actuated by solenoid devices 40 and 42, respectively. The valves are series connected respective to one another and control a flow of compressed fluid from supply pipe 44 into an air inlet tube 45.

Control box 46 of FIG. 1 is connected to each of the before mentioned, solenoid actuated valves and to a suitable source of electrical current S. The control box 45 includes circuitry for accomplishing the manipulation of the valves in a sequence of events necessary for establishing the flow of air and plastic material through the pipe according to the invention.

In FIG. 2, an appropriate quantity of powdered plastic 47, hereinafter called a synthetic resin material, or a "pile", or a "charge", lies dormant within the powder chamber of the housing 36. Spider 48 supports a cone 50 axially within the main housing. Charge door 51 admits a charge 47 into the powder chamber. In order to assure a uniform coating, the charge is slightly greater in weight as compared to the actual amount of plastic required to coat the pipe.

One example of the circuitry 46, disclosed in FIG. 1, is shown in greater detail in FIGS. 2 and 4. As seen in FIG. 2, the circuitry includes current legs 52 and 53 which provide current flow to the solenoids 32 and 38 through the switch means seen at "S" and 55. According to FIG. 2, closure of the main switch at S energizes legs 52 and 53. Closure of switch 55 simultaneously opens valves 31 and 37 which establishes a mass flow through the pipe 18 and moves the charge 47 towards the pipe inlet with the charge becoming a moving pocket of powdered plastic as seen at 147 in FIG. 4. The

flow of air continues uninterrupted through the pipe such that the pocket is pushed through the pipe interior under a positive pressure gradient. The moving pocket is shorter in length than the pipe. The flow of air through the heated, spinning pipe is continued until sufficient time has elapsed for the fused particles to somewhat cool and becomes a continuous, self-supporting plastic film which adheres to the interior wall of the pipe.

The switch 55 is next opened, another charge placed into the chamber, another prepared pipe substituted for the processed one at 16, and the before mentioned sequence of events are then repeated while the last processed pipe is transferred into the soaking oven for post-treatment as required.

As seen in FIGS. 2 and 5, a pipe 18 can be suitably coated in the above described manner without the use of the primary blow air at 45; however, in such an instance, there must be a sufficient volume presented by the interior of the pocket-forming apparatus between the valve 37 and the inlet to pipe 18 for the mass flow to properly accelerate before the pocket reaches the pipe inlet. This is achieved by eliminating the primary blow air as seen in FIG. 2, or by eliminating current flow to the solenoids 40 and 42 of the primary blow air valves 25 so that the injection apparatus at 45 becomes dormant except for the turbulence caused by the outer marginal end portion thereof which is located within the chamber 29.

In FIGS. 2 and 3, the annulus 56 formed between the 30 cone and pocket-forming housing forces the air to flow in a pattern which enhances the charge of plastic at 47 to assume the form of a moving, concentrated pocket of material as it flows towards the adapter.

Looking in greater detail now to the embodiment of FIG. 4, it will be noted that two conductors one of which is seen at 58, are connected to the illustrated source of current "S". Contact 60, when manually closed, energizes a first time delay device 62 which closes contacts 63 thereof for a finite time interval equal to one cycle of operation. Closure of the contacts of TD1 energizes the solenoid 42 which moves the normally closed valve 41 to the open position, and simultaneously energizes the solenoid 64 of TD2. Closure of contacts 66 of TD2 is momentarily delayed for a time 45 interval of less than one second in order for flow through 45 and into the heated, rotating pipe to reach equilibrium. Closure of contacts 66 energizes the solenoid of TD3, thereby closing the contacts 67 which remain closed until the TD3 solenoid is de-energized and thereafter times out.

Closure of contacts 67 simultaneously energizes solenoids 32, 38, and 40 to cause the valves 31 and 37 to move to the open position concurrently with the closure of valve 39 so that mass flow through the apparatus 55 is uninterrupted.

It is necessary that the minimum time interval of either of TD3 and TD1 be set to a value which is sufficient to enable the charge 147 to be flowed through the rotating, heated pipe and for the flow of air to continue through the pipe until the pocket of plastic particles has deposited and fused into a continuous uniform coating therewithin. The cycle of operation ends when TD1 and TD3 time out, thereby returning the valves 31, 37, 39, and 41 to their standby configuration.

The charge of plastic 47 in FIG. 2 is illustrated in FIG. 4 as having been fluidized as it commences to move as a pocket downstream at 147. The pocket at 247

is shown flowing through the heated, rotating pipe 18 while it coats the pipe wall in the manner of FIG. 6. In actual practice, of course, there is only one charge 47, which is changed into only one pocket 147 or 247 as the charge is forced to flow through the pipe.

FIG. 5 is a diagrammatical illustration of another embodiment of this invention. The pocket of plastic material 47 is seen isolated in the charge containing enclosure or chamber by the employment of the before mentioned, two spaced valves 31 and 37 which are series connected respective to one another with the charge being located therebetween. The valves are connected in series with inlet 30 and pipe inlet 78. The inlet 30 is open to the atmosphere, while the outlet 80 is connected to suction-producing apparatus 130, which produces a mass flow through the entire apparatus when the valves 31 and 37 are opened. The charge of plastic becomes fluidized as illustrated at 47 to form the illustrated pocket of plastic 247. For purposes of illustration, the pocket is also shown within the pipe after it has moved from 47 into a marginal length of the pipe interior. As noted in various figures of the drawings, the pocket is not as long as the pipe.

In FIG. 6, the pocket is in the act of flowing through the pipe 18. A coating at 82 has been fused thereon as schematically illustrated therein. As the pocket flows through the pipe, the plastic particles contained therewithin contact and fuse to the pipe wall as illustrated at 83. The purpose of FIG. 6 in conjunction with other figures of the drawings is to illustrate the inventor's concept of the process of the present invention.

In FIG. 7, a plastic-containing enclosure 136 is included as part of the main housing 28 of FIG. 2 for providing a fluidized bed 47. Porous baffle 72 divides the apparatus 136 into a lower air housing 70 and an upper fluidized bed section 74. Air inlet 76 emits a small controlled air flow into housing 70 to establish the fluidized bed. Provision must be made for a small egress of air from the upper end of 74 in order to maintain the fluidized bed while valves 31 and 37 are closed. This can be accomplished by any number of different expedients, including the provision of a small, looped tube which is connected from 74 into the downstream side of valve 37, or alternatively, a small aperture formed through the upper part of the valve seal element.

In operation of FIGS. 1 and 4, a quantity of powdered plastic is charged into the chamber 36. At this time, the valve 31 and 37 are closed, while valve 39 is opened. A source of air pressure is made available at supply inlets 30 and 44. The cleaned, preheated pipe 18 is received at 16 and rotated at a speed of about 100 rpm, depending upon the i.d. of the pipe. The adapter 24 is placed in attached relationship at the inlet end of the pipe 18 so that any subsequent flow of material from the pocket-forming apparatus will be forced to flow from the flexible hose, through the adapter, and into the pipe, with minimal leakage occurring between the adapter and the inlet end of the pipe in order to avoid waste of material. The outlet end of the pipe is left opened to atmospheric pressure.

Primary air flow through tube 45 is initiated by opening the N.C. valve 41 and thereafter both valves 31 and 37 are opened while valve 39 is simultaneously closed. This action produces a continuous mass flow through the pipe during the coating process. During the continuous flow of material, the pocket moves through the pipe with no interruption of flow, and it is believed that this

uninterrupted type of flow contributes to the success of the present process.

In the embodiment of FIG. 2, the primary air seen at 45 in FIGS. 1 and 4 has been eliminated. The outlet end of pipe 18 is open to atmosphere. The charge of plastic is blown through the pipe 18 in the before described manner. The downstream valve 37 can be replaced with a baffle which forms a dam, if desired.

When it is necessary to coat long joints of pipe, the uniformity of the coating thickness can be improved by 10 throttling the air flow so that the pocket enters the pipe at a relatively high velocity and exits the pipe at a relatively low velocity. This can be accomplished by the provision of a control means which varies the rate of flow through the pipe by manipulation of either of the 15 valves 31 or 37. For example, solenoid 32 can fully open the valve 31 to provide a high pressure at 33 and, after the pocket has entered the pipe inlet, the valve can commence to close in proportion to the distance the 20 pocket has traveled through the pipe. Hence, the rate of velocity of the traveling pocket of plastic through the pipe can be employed to enhance the uniformity of the coating thickness.

It has been found that an initial pressure of 19 psig 25 effected at source 30 and progressively reduced to 13 psig as the pocket exits the pipe works to advantage where a difference in coating thickness is noted at each extremity of the processed pipe.

In FIG. 5, an appropriate charge is placed within the pocket-forming apparatus, with the valves 31 and 37 being closed so as to isolate the charge. Suction is applied at the outlet end 80 of the heated, rotating pipe, the valves 31 and 37 opened, whereupon the charge is forced to move through the pipe. Atmospheric pressure only is effected at 30 in FIG. 5.

#### Example I:

Pipe size: 2 $\frac{3}{8}$  I.D.

Length: 31-33'.

Preheat temperature: 375° F.

Powder type: Corvel.

Air pressure at inlet 30: 19 psi.

Type: J55 tubing.

Rotational speed: 135 rpm.

Ounces employed: 32.

#### Example II.

Pipe size: 2 $\frac{3}{8}$  I.D.

Length: 31-33'.

Preheat temperature: 375° F.

Powder type: Corvel.

Air pressure at inlet 44: 19 psi.

Air pressure at inlet 30: 19 psi.

Type: J55 tubing.

Rotational speed: 135 rpm.

Ounces employed: 32.

I claim:

1. Method of powder coating the interior of individual joints of pipe with a powdered synthetic resin material, comprising the steps of:

- (1) preheating each of the joints of pipe to a temperature in excess of the fusion temperature of the synthetic resin material;
- (2) successively rotating each of the preheated joints of pipe about its longitudinal axis at a speed which enables any subsequently fused synthetic resin material to spread into a continuous film about the interior of the joints of pipe;
- (3) making a pocket-forming apparatus by forming a chamber within which a charge of powdered syn-

thetic resin material can be isolated; providing said chamber with an inlet end and an outlet end; and, connecting one end of a rotating joint of pipe to the outlet end of the chamber; and, applying atmospheric pressure to the inlet end of the chamber;

- (4) placing a dormant charge of powdered synthetic resin material within the chamber of said pocket-forming apparatus; said dormant charge being in excess of the amount of powdered resin material required to uniformly coat the entire interior of said rotating joint of pipe in a single pass of the dormant charge through the rotating joint of pipe;
- (5) forming from said dormant charge a pocket of powdered synthetic resin material which is smaller in volume than the interior of said rotating joint of pipe; and, forcing said pocket to move into the interior of said rotating joint of pipe by applying a suction at the other end of the rotating joint of pipe; thereby forcing a stream of compressible fluid to flow through the inlet end of the chamber of said pocket-forming apparatus to substantially simultaneously move the entire dormant charge from the chamber into said rotating joint of pipe as the pocket of powdered resin material, whereupon the interior of said preheated, rotating joint of pipe is coated with synthetic resin material contained within the pocket in a single pass of the pocket therethrough;

(6) said pocket, as it flows through the interior of said joint of pipe, is limited to a length which is less than the length of said joint of pipe.

2. The method of claim 1 wherein said pocket-forming apparatus is provided with a valve means upstream of said inlet end of said chamber, so that when a suction is applied to the other end of the pipe joint and the valve means is opened, said dormant charge moves from said pocket-forming apparatus into said joint of pipe as a dense pocket comprised of a mixture of air and plastic powder.

3. Method of powder coating the interior of a pipe with a powdered synthetic plastic resin material comprising the steps of:

- (1) preheating the pipe to a temperature in excess of the fusion temperature of the powdered plastic resin;
- (2) rotating said preheated pipe of step (1) about its longitudinal axis at a velocity which causes any subsequently fused plastic material to spread out into a continuous film;
- (3) said pipe has an inlet end opposed to an outlet end; connecting an inlet end of the pipe to one end of a flow conduit, while the other end of the pipe is connected to a source of reduced pressure;
- (4) placing a charge of the plastic powder upstream of the pipe inlet and within the flow conduit; said charge lies dormant within said flow conduit, the dormant charge being in excess of the quantity of plastic required to coat the interior of the pipe;
- (5) applying atmospheric pressure to the other end of the flow conduit at a location upstream of said dormant charge to cause a pressure differential across the entire dormant charge which is of a magnitude to form the entire dormant charge into a fluidized pocket of plastic material having a volume which is less than the volume of the interior of the pipe, the pressure differential being of a magnitude to move the pocket into and along the length of the pipe; and,

(6) continuing to effect said pressure differential to move the entire pocket from the flow conduit and through the preheated, rotating pipe, while limiting the length of the pocket to a value less than the length of the pipe; whereupon said pocket progressively deposits particles of powdered plastic onto the heated, inside surface of the pipe, and the particles of plastic fuse thereto as the pocket moves into the pipe inlet, through the pipe, and out the other end of the pipe.

4. Method of powder coating the interior of a single joint of large, long, pipe with a powdered synthetic plastic resin comprising the steps of:

- (1) selecting a synthetic plastic resin material in particulate form which is capable of being bonded to the interior wall surface of a large, long, heated joint of pipe;
- (2) preheating the joint of pipe to a temperature in excess of the fusion temperature of the powdered synthetic resin material;
- (3) rotating the preheated joint of pipe about its longitudinal axis at a speed which enables any subsequently fused resin material to spread onto the interior wall surface of the joint of pipe as a continuous film;
- (4) providing a chamber with an inlet and an outlet; and isolating a charge of the resin material of step (1) within said chamber; said charge lying dormant within said chamber, the dormant charge being in excess of the amount of powdered plastic resin material required to uniformly coat the interior wall surface of said joint of pipe;
- (5) communicating one end of the rotating, preheated, joint of pipe with the outlet of said chamber;

5

10

ber, while connecting the other end of the joint of pipe to a suction means to cause a reduced pressure between the interior of the joint of pipe and the atmosphere;

(6) forming the dormant charge of plastic resin material into a dense pocket which is smaller in volume than the interior of said joint of pipe by forcing the entire dense pocket of step (4) to flow into the interior of said joint of pipe by applying said suction means whereupon a pressure differential is effected across the pocket as a stream of compressible fluid from the atmosphere flows through the inlet of said chamber and through said joint of pipe, thereby forming the pocket with the leading part of the stream of compressible fluid, and moving the pocket only one time through the joint of pipe in advance of the trailing part of said stream of compressible fluid whereupon the interior of said joint of pipe is contacted by and coated with the plastic resin material in a single pass;

(7) said pocket, as it flows through the interior of said joint of pipe is confined to a length which is less than the length of said joint of pipe.

5. The method of claim 4 and further including the step of providing said inlet of said chamber with a valve means; connecting the upstream side of said valve means to a source of atmospheric pressure; forming a moving pocket of plastic material by opening said valve means whereupon a flow occurs through said pocket-forming apparatus and said pocket is moved through said joint of pipe as particles therefrom contact and fuse to the inner wall of the joint of pipe.

\* \* \* \* \*

35

40

45

50

55

60

65